

# United States Patent [19]

[ 19 ]

[11] 3,909,313

Kato et al.

[45] Sept. 30, 1975

- [54] **METHOD FOR FORMING AN ELECTRIC INSULATING FILM HAVING EXCELLENT PUNCHING PROPERTY AND HEAT RESISTANCE ON AN ELECTRICAL STEEL SHEET**

[75] Inventors: **Hirotada Kato; Kazuo Nakamura**, both of Kitakyushu, Japan

[73] Assignee: **Nippon Steel Corporation**, Japan

[22] Filed: **Sept. 21, 1973**

[21] Appl. No.: **399,625**

[30] **Foreign Application Priority Data**  
Sept. 29, 1972 Japan ..... 47-97777

[52] U.S. Cl. ..... **148/113; 117/230; 117/234; 148/31.5; 148/6.2**

[51] Int. Cl.<sup>2</sup> ..... **H01F 1/04**

[58] **Field of Search** ..... **148/113, 6.2, 6.16, 31.5, 148/122, 6.15; 117/230, 234**

3,477,881 11/1969 Wada et al. .... 148/6.2  
3,523,837 8/1970 Pavlik ..... 148/113  
3,562,011 2/1971 Hirst et al. .... 148/113  
3,649,372 3/1972 Imai et al. .... 148/6.16  
3,785,882 1/1974 Jackson ..... 148/113  
3,793,073 2/1974 Kitayama et al. .... 117/230

*Primary Examiner*—Walter R. Satterfield  
*Attorney, Agent, or Firm*—Toren, McGeady and Stanger

[57] **ABSTRACT**

A method for forming on an electrical steel sheet an electric insulating film having excellent punching property and heat resistance comprising coating on the steel sheet a treating solution comprising a composition composed of one or more of chromic anhydride, chromate, bichromate and 1 – 35 parts (as solid) of styrene resin containing not less than 50% styrene and/or vinyl acetate resin emulsion per 10 parts of chromic anhydride in the composition and heating the coating.

## References Cited

UNITED STATES PATENTS

- 3,389,006 6/1968 Kohler ..... 148/113

## ABSTRACT

A method for forming on an electrical steel sheet an electric insulating film having excellent punching property and heat resistance comprising coating on the steel sheet a treating solution comprising a composition composed of one or more of chromic anhydride, chromate, bichromate and 1 - 35 parts (as solid) of styrene resin containing not less than 50% styrene and/or vinyl acetate resin emulsion per 10 parts of chromium ion in the composition and heating the coating at a temperature between 150° and 500°C.

## 5 Claims, 2 Drawing Figures

FIG. 1



FIG. 2



**METHOD FOR FORMING AN ELECTRIC  
INSULATING FILM HAVING EXCELLENT  
PUNCHING PROPERTY AND HEAT RESISTANCE  
ON AN ELECTRICAL STEEL SHEET**

The present invention relates to a method for forming an electric insulating film having excellent punching property and heat resistance on the surface of an electrical steel sheet. The electrical steel sheet used herein includes all of so called silicon steels and low carbon steels usable for iron cores of electrical appliances.

It is well known that silicon steel sheets or low carbon iron plates in which impurities, such as, carbon is reduced as low as possible have been used for electrical instruments, such as, transformers and generators.

The electric insulating film coated on the electrical steel sheets is required to have excellent inter-layer resistance, film adhesion, corrosion resistance, weldability and punching properties in addition to electric insulating properties.

The punching property of the electrical steel sheet has an important influence on the dies for punching the sheet, and excellent punching property assures increased number of punchings per one die and thus considerably elongates the life of the die.

The punching property can be improved to some degree by material improvement of the electrical sheet itself, but there is a limitation to the degree of improvement that can be effected by this alone.

The present invention will be described in detail by referring to the attached drawings.

FIG. 1 is a graph showing the relation between the additional amount of styrene resin and the punching property, and

FIG. 2 is a graph showing the relation between the burr height and number of punchings in the comparison 1 and Examples 2 and 3.

The present inventors have found that the punching property is largely influenced by the electric film formed on the surface of the electrical steel sheet and have conducted various extensive studies on the basis of the discovery, and have succeeded in developing film agents which make possible to increase the number of the punchings per one die to 2,500,000 that is, 5 to 30 times as compared with the conventional insulating film, and a method for forming the film.

The conventional film agent, for example, an insulating film formed with a treating solution prepared by mixing divalent metal oxides with chromic acid anhydride shows the punching property as shown by the curve (a) in FIG. 2, where with about 80,000 punchings, burrs reach 50 $\mu$  of the allowable limit.

Further, heat resistance is one of the important properties of the electric insulating film. Generally, heat treatment of the electrical steel sheets is done in the piled form in order to remove the working strain and improve magnetic characteristics, and is usually done in a neutral or weak-reducing atmosphere, depending on the purposes of the treatment. In this case, heat resistance, namely, non-peeling of the insulating film is required.

Further, since generators for refrigerator compressors use freon gas if on the exposed edge surface of the iron core made by punching the electrical steel sheet, rust is formed and the rust strips off, it can get into the gas and clog the expansion valve. Further the exposed

metal serves as a catalyst and decomposes the freon gas. In order to solve such problems, the punched edge surface is subjected to a blueing treatment. In this treatment also, it is required that the insulating film not peel off; powdering does not occur at the treating temperature between 400° and 600°C, and the piled sheets do not adhere to each other. Thus an additional type of heat resistance is required.

Therefore one purpose of the present invention is to provide an electric insulating film for an electrical steel sheet, which film does not undergo thermal deterioration which cause the above troubles during the heat treatments, and which also possesses remarkably improved punching properties.

The steel plate sheet or strip to which the present insulating film is applied include silicon steel plates or low carbon iron plates containing very small amounts of silicon or containing no silicon which are generally used for electrical appliances, such as, generators and transformers.

As the insulating film agents for the electrical steel plate, a mixture of chromate and resin emulsion is known as disclosed in Japanese patent publication Sho 40-6722.

In general, when the treating solution of chromic acid with the addition of resin emulsion is coated and baked on the steel plate, the agent serves as a good solid lubricant and gives good punching property because of the small emulsion particles (0.1 to 1 $\mu$ ).

However, when most of the above resin emulsions are added to the chromic acid solution, the resin particle is broken and instantly gels or gradually gels and produces sediment.

Further, when the above treating solution is applied on the steel plate by rolls, the sediment adheres to the rolls and thus a uniform film can not be obtained.

Meanwhile, when commercially available emulsion resins, such as, vinyl acetate emulsion using PVA protection colloids for paints, acrylic acid ester emulsion, or ethylene vinyl acetate emulsion are added to the chromic acid solution and the thus prepared treating solution is applied on the electrical steel plate, only poor heat resistance is obtained and the film peels off or powders during the heat treatment.

Therefore, another object of the present invention is to provide a method for forming an electric insulating film which has overcome the above defects.

The treating solution for forming the film according to the present invention may be prepared by adding styrene resin to a composition (A) containing one or more of chromic anhydride, chromate and bichromate.

As for the chromate or bichromate of the above composition (A), salts of bivalent metals, such as, magnesium, calcium and zinc, may be used.

Also, an aqueous solution prepared by dissolving oxides of bivalent metals, such as, MgO, CaO, ZnO; hydroxides, such as, Mg(OH)<sub>2</sub>, Ca(OH)<sub>2</sub> and Zn(OH)<sub>2</sub>, or carbonates, such as, MgCO<sub>3</sub>, CaCO<sub>3</sub> and ZnCO<sub>3</sub> in chromic anhydride in an amount less than their dissolution limit may be used. This aqueous solution composition may be considered to be an aqueous solution of a mixture of chromic anhydride and chromate. When the above oxide, hydroxide or carbonate of the bivalent metal ion is added to the dissolution limit, the heat resistance of the film lowers, and the film peels off during the strain-relief annealing step and the blueing step. Further, when these additions are added in an amount

60

more than their dissolution limit, non-dissolved powders are applied together with the treating solution so that the surface luster is lost and the film easily peels off near the edge surface during the stamping of cores.

As for the styrene resin to be added to the composition (A), styrene emulsion resin, styrene-acryl copolymer emulsion, and styrene vinyl acetate resin may be used.

In case of a copolymer of the styrene resin and other resins, it is required that styrene is contained in an amount of 50% or more as solid component. If the proportion of styrene is less than 50%, the heat resistance is poor so that the film will peel off or powder during the heat treatment.

On the other hand, a mixture of styrene emulsion and emulsion of other resins also can give satisfactory heat resistance.

The proportion of the styrene emulsion to the composition (A), for example, to chromic anhydride, is 1 to 35 parts to 10 parts of chromium ions contained in the chromic anhydride. With less than one part addition of the styrene resin, no effect is obtained by the addition and the desired punching property can not be obtained. On the other hand, if the addition is over 35 parts, the punching property is not improved any further, but the film softens during the heating and is easily damaged.

Further, poor conductor-forming oxides, such as, boric acid, colloidal silica, colloidal alumina, sodium silicate and potassium silicate may be added to the treating solution used in the present invention without deviating from the scope of the present invention.

The above oxides, however, should be added in a range from 2 to 16 parts to 10 parts of the chromium ions in the composition (A).

The water-soluble saturated dicarboxylic acids having four or more carbon atoms used in the present invention are acids, such as, succinic acid, adipic acid, glutamic acid, and pimelic acid. For the reduction of hexavalent chrome, the above carboxylic acid is used, and when other carboxylic acids are used, the following defects arise.

For example, with mono-carboxylic acids, such as, formic acid and acetic acid, the reducing force is so large that the reduction is effected in such a degree as to precipitate the inorganic substances and of the emulsion resin, thus damaging the stability of the solution, and result in a film having poor appearance, adhesion and heat resistance. Further, when saturated carboxylic acids such as, oxalic acid having two carbon atoms are used, a good film is not obtained, and with the use of nonsaturated carboxylic acids, such as, maleic acid, the stability of the solution is poor. Only when saturated carboxylic acids having 4 or more carbon atoms are used is the stability of the inorganic substances and the emulsion very excellent and a good film for an electrical steel sheet can be obtained.

Polyethylene glycols having about 200 to about 1000 molecular weight are most preferable for use in the present invention. Ethylene glycol has so strong a reducing force that the solution stability is not obtained, and similarly polyhydric alcohols, such as, glycerine, amines, such as, triethanolamine, are not usable as they promote settlements of inorganic substances and of the emulsion resins.

The optimum proportion of the water-soluble saturated carboxylic acid having 4 or more carbon atoms

and the polyethylene glycol is from 1 to 10 parts to 10 parts of the chromium ion. With less than 1 part, the reducing force is low and a large amount of hexavalent chromium remains in the film and the film dissolves in water. Even with more than 10 parts, the effects of the reducing agent will not change substantially.

The treating solution having the above composition may be applied on an electrical steel plate having suitable surface conditions by any of the conventional coating methods, such as, roll coating, brushing, spraying and immersion.

Although there is no special limitation in the coating amount of the treating solution, it is most desirable that the residual solid substance after the heating and baking is 0.5 to 5 g/m<sup>2</sup>.

According to the present invention, the baking after the coating of the treating solution is done at a steel surface temperature of 150° to 500°C and the heating time for the baking is not specifically limited, but a heating time between 10 and 180 seconds will give good results.

When the heating temperature is lower than 150°C, no satisfactory baking is obtained and the film has no water-resistance and becomes viscous by absorption of water. On the other hand, when the heating temperature is higher than 500°C, the film agent is decomposed and thus the film adhesion and the punching property become poor thus failing to obtain the desired results of the present invention.

The electric insulating film formed by the method of the present invention is excellent in both of the punching property and heat resistance, and the solution itself has good stability and can stand for long time.

The styrene emulsion resin is prepared by polymerization under the presence of an emulsifying agent (mainly a surface activating agent), and the stability of the emulsion resin in the treating solution of the present invention is influenced by the kind of the emulsifying agent to used. When an anionic activating agent, for example, laulylic sodium sulfate is used, the emulsion resin readily settles in a short time. Nonion activating agents (for example, polyoxyethylene nonyl phenyl ether, polyoxyethylene alkyl-aryl ether) or nonion-anion mixture activating agents (for example, a mixture of polyoxyethylene noel phenol ether and dodecylbenzene sulfoninate) are preferable.

By using the above specified reducing agents (saturated carboxylic acids having 4 or more carbon atoms and polyethylene glycol) and styrene emulsion resins polymerized under the presence of nonion activating agents or nonion-anion mixture activating agents, the settlement and gellation of the emulsions is effectively prevented and the emulsions can be preserved for more than one month.

The vinyl acetate emulsions used in the present invention should be polymerized using nonion activating agents or nonion-anion mixture activating agents, and the vinyl acetate emulsions which are polymerized using high-molecular protection colloids, such as, commercially available PVA and cellulose derivatives for paints, should be avoided. When the latter emulsions are used, not only is the solution stability is poor, but also thermal deterioration is observed during the heat treatment and the film easily peels off after the strain-relief annealing and the blueing treatment. These defects are not observed when the former vinyl acetate resins are used.

Therefore, the vinyl acetate emulsion resins in the present invention means the vinyl acetate emulsion resins and the vinyl acetate-acryl copolymerization emulsion prepared by using the above activating agents.

The present invention will be more clear from the following examples.

### EXAMPLE 1

Treating solutions prepared by adding 2 parts, 5 parts, 15 parts, 20 parts and 30 parts of styrene-acryl copolymerization emulsion (total solid components 40%, acryl 10% in the solid components) to the composition A comprising 20 parts of chromic anhydride (chrome ion 10 parts), 6 parts of magnesium oxide, 2 parts of adipic acid (reducing agent) and 250 parts of water were coated by rolls uniformly on an electrical steel sheet, heat-treated at a sheet temperature 350°C to form a uniform insulating film in an amount of 2 g/m<sup>2</sup>.

The characteristics and punching property of the film are shown in Table 1. The stability of the above treating solutions were very excellent and no settlement was observed after more than one month.

### EXAMPLE 2

A treating solution having the following composition:

|                                    |           |
|------------------------------------|-----------|
| Chromic anhydride                  | 20 parts  |
| Zinc oxide                         | 8 parts   |
| Boric acid                         | 8 parts   |
| Ethylene glycol (reducing agent)   | 2 parts   |
| Styrene emulsion (solid component) | 10 parts  |
| Water                              | 300 parts |

was coated by rolls on a silicon steel sheet, heated at a sheet temperature of 280°C to form a film in an amount of 2.6 g/m<sup>2</sup>, whose characteristics are shown in Table 1.

### EXAMPLE 3

A treating solution having the following composition:

|                                                                  |        |
|------------------------------------------------------------------|--------|
| Chromic anhydride                                                | 25 Kg  |
| Magnesium oxide                                                  | 7.5 Kg |
| Boric acid                                                       | 10 Kg  |
| Succinic acid (reducing agent)                                   | 1.8 Kg |
| Styrene acryl emulsion (solid component)                         | 35 Kg  |
| (solid component 40%, ratio of styrene to ethylacrylate 55 : 45) |        |
| Water                                                            | 400 l  |

was left at ordinary temperatures for 15 days and then coated by rolls on an electrical steel sheet and baked at a sheet temperature of 300°C, thereby a lustrous and uniform film was formed on the steel sheet in an amount of 1.8 g/m<sup>2</sup>. No gellation of the solution and no settlement were observed.

### EXAMPLE 4

A treating solution having the following composition:

|                                                                       |        |
|-----------------------------------------------------------------------|--------|
| Calcium chromate                                                      | 25 Kg  |
| Chromic anhydride                                                     | 12 Kg  |
| Boric acid                                                            | 6 Kg   |
| Succinic acid                                                         | 4.5 Kg |
| Styrene acryl copolymerization emulsion                               | 25 Kg  |
| (resin solid 40%, ratio of styrene to butyl acrylate 9 : 1 by weight) |        |
| Water                                                                 | 400 l  |

was left at ordinary temperatures for 1 month and then coated by rolls on an electrical steel sheet, and heated at a furnace temperature of 500°C for 35 seconds, thereby a uniform and lustrous film was formed on the steel sheet in an amount of 2.3 g/m<sup>2</sup>. The solution was stable and no settlement was observed.

### EXAMPLE 5

A treating solution having the following composition:

|                                            |        |
|--------------------------------------------|--------|
| Chromic anhydride                          | 20 Kg  |
| Magnesium oxide                            | 5 Kg   |
| Boric acid                                 | 5 Kg   |
| Succinic acid                              | 2 Kg   |
| Polyethylene glycol (molecular weight 400) | 2 Kg   |
| 40% polystyrene emulsion resin             | 10 Kg  |
| 40% vinyl acetate emulsion                 | 10 Kg  |
| Water                                      | 300 Kg |

was left at ordinary temperatures for 1 month and then coated by rolls on an electrical steel sheet and heated at a sheet temperature of 300°C, thereby a uniform and lustrous film was formed on the sheet in an amount of 2.1 g/m<sup>2</sup>. No gellation of the solution and no settlement were observed. The punching property test showed 1,200,000 times and the adhesion property test showed less than 10mm. The results of the corrosion resistance test and the heat resistance test were similar as those of the other examples.

### EXAMPLE 6

A treating solution having the following composition:

|                                                   |        |
|---------------------------------------------------|--------|
| Chromic anhydride                                 | 20 Kg  |
| Magnesium oxide                                   | 6 Kg   |
| Boric acid                                        | 4 Kg   |
| Succinic acid                                     | 4 Kg   |
| 40% vinyl acetate acryl copolymerization emulsion | 30 Kg  |
| (ratio of vinyl acetate to butyl acrylate 7 : 3)  |        |
| Water                                             | 300 Kg |

was left at ordinary temperatures for one month and then heated at a sheet temperature of 300°C, thereby a uniform and lustrous film was formed on the sheet in an amount of 2.1 g/m<sup>2</sup>. No gellation of the solution and no settlement were observed. The punching property test showed 1,600,000 times and the adhesion property test showed less than 10 mm. The corrosion resistance and the heat resistance test were similar as those in other examples.

Table 1.

| Ex.<br>No. | Treating Solution                   | Punching property and film characteristics |                         |
|------------|-------------------------------------|--------------------------------------------|-------------------------|
|            |                                     | Punching<br>property *1<br>(in thousand)   | Adhesion<br>Property *2 |
| 1          | A Solution + Styrene Resin<br>parts |                                            |                         |
|            | 2.5                                 | 200                                        | 20 φ                    |
|            | 5                                   | 600                                        | 10                      |
|            | 10                                  | 1200                                       | less than 10            |
|            | 15                                  | 1600                                       | "                       |
|            | 20                                  | 2050                                       | "                       |
|            | 35                                  | 2400                                       | "                       |
| 2          |                                     | 1350                                       | "                       |
| 3          |                                     | 2300                                       | "                       |
| 4          |                                     | 1800                                       | "                       |

Table 1 -Continued

| Ex.<br>No.         | Treating Solution                               | Punching property and film characteristics |                            |
|--------------------|-------------------------------------------------|--------------------------------------------|----------------------------|
|                    |                                                 | Punching<br>property *1<br>(in thousand)   | Adhesion<br>Property *2    |
| <b>Comparative</b> |                                                 |                                            |                            |
| 1                  | A Solution                                      | 80                                         | 20 $\phi$                  |
| 2                  | A Solution + Vinyl Acetate Resin *3<br>15 parts | 1400                                       | 30 $\phi$                  |
| 3                  | A Solution + Acryl Resin<br>10 parts            | 1050                                       | 20 $\phi$                  |
| Heat Resistance *5 |                                                 |                                            |                            |
| Ex.<br>No.         | Corrosion<br>Resistance<br>*4                   | Stress-relief<br>Cloth                     | Annealing<br>Vinyl<br>tape |
|                    |                                                 | Good                                       | No peeling                 |
| 1                  | Good                                            | Good                                       | Blueing<br>Vinyl<br>tape   |
| "                  | "                                               | "                                          | "                          |
| "                  | "                                               | "                                          | "                          |
| "                  | "                                               | "                                          | "                          |
| 2                  | "                                               | "                                          | "                          |
| 3                  | "                                               | "                                          | "                          |
| 4                  | "                                               | "                                          | "                          |
| <b>Comparative</b> |                                                 |                                            |                            |
| 1                  | Slightly<br>bad                                 | "                                          | "                          |
| 2                  | "                                               | Bad                                        | Complete<br>peeling        |
| 3                  | Good                                            | Bad                                        | Partial<br>peeling         |
|                    |                                                 |                                            | Complete<br>peeling        |
|                    |                                                 |                                            | Partial<br>peeling         |

\*1 Punching property: Number of punchings up to the burr allowance limit of 50 $\mu$ .

\*2 Adhesion property: Diameter of the smallest arc which peels off when the sheet is bent in a predetermined arc (180°) and bent back.

\*3 Commercially available polyvinyl alcohol protection colloids are used.

\*4 Corrosion resistance: Rust formation and viscous film after 48 hours immersion in a moistened tank (50°C)

\*5 Heat resistance: Strain-relief annealing at 760°C for 3 hours in N2. Blueing at 560°C for 2 hours with vapour blowing. "Cloth" means the surface was rubbed with gauze ten times. "Vinyl tape" means a vinyl tape was attached to the surface and peeled off.

The comparisons in Table 1 show the results obtained by coating the following solutions (1) (2) (3) by rolls on the steel sheet and heating at 300°C to form a film in an amount of 2 g/m<sup>2</sup>.

|              |                                                                               |
|--------------|-------------------------------------------------------------------------------|
| Solution (1) | only the composition A                                                        |
| Solution (2) | the composition A + 15 parts as solid of vinyl acetate emulsion (solid 50%)   |
| Solution (3) | the composition A + 10 parts as solid acrylic acid ester emulsion (solid 40%) |

The vinyl acetate emulsion, the acrylic acid ester emulsion of the comparisons had poor stability and settlements were observed in 1 day in the former and in 4 days in the latter.

As clearly understood from Table 1, the film adhesion, corrosion resistance and heat resistance are all excellent in the present invention.

What is claimed is:

1. A method for forming an insulating film having excellent punching and heat resistant properties on the surface of an electrical steel sheet comprising applying to an electrical sheet, a composition consisting essentially of chromic anhydride, a chromate of a bivalent metal or a bichromate of a bivalent metal; 1 to 10 parts per ten parts on a weight basis of a reducing agent se-

lected from the group consisting of saturated dicarboxylic acids having 4 or more carbon atoms and polyethylene glycol; and 1 to 35 parts of an aqueous emulsion of a styrene resin containing at least 50% on a solids basis of styrene or an aqueous vinyl acetate emulsion prepared using a nonionic or mixture of a nonionic and anionic activating agent, the vinyl acetate emulsion being prepared in the absence of a high molecular weight protective colloid; and then baking the sheet at a temperature of 150° to 500°C.

2. A method for forming an electric insulating film as claimed in claim 1, wherein the saturated dicarboxylic acid is adipic acid, succinic acid, pimelic acid or glutaric acid.

3. A method for forming an electric insulating film as claimed in claim 1, wherein the polyethylene glycol has a molecular weight from 200 to 1000.

4. A method for forming an electric insulating film as claimed in claim 1, wherein the aqueous styrene resin emulsion containing 50% or more of styrene is a styrene emulsion, a styrene-acrylic copolymer emulsion or a styrene-vinyl acetate emulsion.

5. A method for forming an electric insulating film as claimed in claim 1, wherein the aqueous vinyl acetate emulsion is a vinyl acetate emulsion or a vinyl acetate-acryl copolymer emulsion.

\* \* \* \* \*